

3,834,977

**SHOCK-PROOF NYLON CARPET SYSTEM**  
Ronald Edward Rothwell, Colonial Heights, Va., Cipriano Cipriani, Morristown, N.J., and Julian Lee Rush, Richmond, Va., assignors to Allied Chemical Corporation, New York, N.Y.  
No Drawing. Filed Mar. 29, 1972, Ser. No. 239,378  
Int. Cl. D03d 27/00

U.S. Cl. 161—67

8 Claims

## ABSTRACT OF THE DISCLOSURE

A shock-proof carpet system having a face yarn of textured nylon containing up to about twelve weight percent of an internal additive selected from ethylene oxide condensation products, a primary backing of jute or spun-bonded synthetic material, a tuft-locking latex made electrically conductive by the additive of up to about ten weight percent of an antistatic material, and a standard secondary backing.

## CROSS REFERENCE TO RELATED APPLICATION

This application is related to copending application, Ser. No. 185,816, filed Oct. 1, 1971, by Lamberto Crescentini and Gene Clyde Weedon, now abandoned, in favor of continuation-in-part Ser. No. 239,905, filed Mar. 31, 1972, which was abandoned in favor of continuation-in-part Ser. No. 274,971, filed Oct. 11, 1972, and is hereby incorporated by reference into this application.

## BACKGROUND OF THE INVENTION

This invention relates to a shock-proof carpet system based on nylon. More particularly it relates to an improved carpet system based on nylon made shock-proof by use of certain additives. And, still more particularly it relates to a carpet system based on nylon made shock-proof by use of additives that actually improve its shock-proofness as the carpet system wears.

Carpet systems are well known to generate considerable charges of static electricity when a person in contact therewith traverses the carpet system's fibrous layer. Such charges are quite naturally transferred to the person traversing said carpet system and upon grounding, the charges are discharged causing momentary shock and a source of considerable irritation. And, although several carpet systems have been devised in an effort to improve this system, all tend to become less and less viable with use. One such static-discharging floor covering system is disclosed in U.S. Pat. 2,302,003 wherein a coating of a flexible electrically coating material, such as a rubber compound containing carbon black, is affixed to the under side of a rug, and a plurality of electrically conducting elements, such as cotton cords, and an electrically conductive rubber composition are used which come into contact with the coating and thus extend to substantially the top of the rug. Another more recent approach to solving this problem of static charge buildup in a carpet system is described in U.S. Pat. 3,288,175, wherein up to about 10% by weight on a continuous carpet system is comprised of metallic fibers in continuous metal to metal contact that have the functional and aesthetic properties of nonmetallic textiles yet possess metallic electrical conductivity thus dissipitating the normal static charge buildup. Still another approach to the solution of this static buildup problem is described in U.S. Pat. 3,510,386.

A prime object of this invention is to provide a shock-proof carpet system. Another object of this invention is to provide a shock-proof nylon carpet system. A further

object of this invention is to provide a shock-proof nylon carpet system wherein the additives utilized in making such carpet system are maintained in the carpet system throughout the life of the carpet system. A still further object of this invention is to provide a shock-proof nylon carpet system wherein the static electricity buildup is lower than the threshold of sensitivity to humans. And, a still further object of this invention is to provide a shock-proof nylon carpet system wherein the static electricity buildup gets actually lower or improves its shock proof effectiveness with normal use. Other objects will appear hereinafter as the description of the invention proceeds.

The above and other objects of this invention are accomplished in preparing an antistatic textile article comprising a fibrous textile layer of the pile type, said pile being prepared from a polyamide fiber containing between about 1% and about 12% by weight of a predominantly branched, chain-extended polymer of the reaction product of a compound represented by the formula:



where  $a$ ,  $b$ ,  $c$ ,  $d$ ,  $w$ ,  $x$ ,  $y$ , and  $z$  are each a whole number and  $R$  is a difunctional radical from a hydrocarbon containing 1 to 13 carbon atoms, and at least one compound selected from the group consisting of diepoxides and compounds which yield the following divalent radicals:



where  $R'$  is a difunctional radical derived from aromatic, heterocyclic, cycloaliphatic or aliphatic hydrocarbons or combinations of them having said fibrous pile secured to a primary backing, and an adhesive conductive latex backing added thereto. The adhesive conductive latex is made conductive by containing up to ten weight percent of said latex from a compound selected from the group consisting of the reaction product of a compound represented by the formula:



where  $a$ ,  $b$ ,  $c$ ,  $d$ ,  $w$ ,  $x$ ,  $y$ , and  $z$  are each a whole number and  $R$  is a difunctional radical from a hydrocarbon containing 1 to 13 carbon atoms, and at least one compound selected from the group consisting of diepoxides and compounds which yield the following divalent radicals:



where  $R'$  is a difunctional radical derived from aromatic, heterocyclic, cycloaliphatic or aliphatic hydrocarbons or combinations of them having said fibrous pile secured to a primary backing, and an adhesive conductive latex backing added thereto and polyethylene oxide.

The antistatic-fiber of this invention can contain certain conventional additives without any adverse effects upon the overall shock-proof carpet system of this invention. That is, the carpet system of this invention is compatible in all instances with other additives, naturally either necessary or desirable, such as, dyeing assists and

colorants, stabilizers, antioxidants and delustrants among others.

Surprisingly, such improved shock-proof carpet system of this invention not only provides a shock-proof carpet system initially below the threshold of sensitivity to humans, but actually improves its shock-proof effectiveness with use. Such threshold of sensitivity to humans has been established at between approximately about 2500 to about 4000 volts. See *Modern Textiles*, April 1971 publication, article "A Shock-Free Carpet System At 10% Relative Humidity" and papers of the American Association For Textile Technology, Inc.® by D. H. Martin, R. D. Radford and K. R. Lea. Another static test procedure for textiles is described in technical bulletin No. 2-015, dated 3/1/70 by Brunswick Corporation, Technical Products Div., 69 W. Washington St., Chicago, Ill 60602. These publications also illustrate the walk-test method employed in static electricity buildup evaluation. These test methods are somewhat redundant, but do complement each other to a great extent. They do agree that a static level greater than about 3 kilovolts or 3000 volts, as measured by these tests, will produce a shock detectable by most people and objectionable to some.

The principles of practicing the invention are further illustrated by the following examples, but without limiting the invention to the details thereof.

#### Example 1

Polycaproamide polymer is used having a moisture content of 0.05% to 0.10%, total constituents extractable by hot water of 1% to 2%, and formic acid relative viscosity of 62. The polymer contains about 0.2% titanium dioxide dulling agent, antioxidant, and 6% of an antistatic agent consisting of a polyether of dimethylterephthalate and Tetronic 1504 supplied by Wyandotte and covered under U.S. Pat. 2,979,528 by Lunsted. The Tetronic 1504 is one of many tetrol compounds commercially available as tetronic series block copolymers having molecular weights between 1650 and 26,000. This series varies in length of poly(oxyethylene) chain and poly(oxypropylene) chain. A 3 and 4 digit code number indicates the molecular composition. When four digits are employed, the first two explain the average molecular weight of the hydrophobe (poly(oxypropylene) branches on the alkylene diamine). When three digits are used only the first number serves this purpose. The last digit of each code number represents the weight percentage of hydrophilic (poly(oxyethylene) units to the nearest 10%). The antistatic material is metered at the hopper with the polycaproamide polymer and both are fed into a screw extruder having an exit temperature of 260° C. The polymer is forwarded at a pressure of 1900 p.s.i.g. through a sand filter to a spinnerette plate with 70 holes, each of which is 0.95 inch deep and 0.025 inch in diameter. The freshly extruded filaments descend a spinning tower into which is air conditioned at 70° F. and 65% relative humidity is admitted. The yarn emerging from the spinning tower contacts a ceramic roll which applies a lubricant finish, and the yarn then is wound onto a package at 1850 feet per minute. The yarn thus obtained has a denier of 3150, is drawn over a 5/8 inch diameter draw pin at a delivery rate of 1536 feet per minute which is 3.01 times the feed rate in order to obtain a drawn yarn denier of 1050 denier. Each of the 70 filaments has a denier of 15. During drawing the yarn is passed 5 wraps over a shoe-type heater maintained at 175° C. The yarn is then subjected to a continuous stuffer box crimping operation and two ends of 1050 denier are combined and twisted together to produce a 2250 denier, 140 filament with a 3/4 "S" type twist yarn.

The yarn is then employed in making a level loop pile tufted carpet having twenty ounces of fiber per square yard of carpet and employing a spun-bonded polypropylene backing scoured, dyed at 212° F., rinsed and dried. The carpet is then double backed with a latex consisting

of styrene butadiene rubber having five weight percent of low molecular weight polyethylene oxide antistatic material. The antistatic properties of this carpet as determined by the Walk Test method wherein the temperature is controlled at 71° F. and the relative humidity is controlled at 20% are compared in Table I with control carpets.

TABLE I

| Sample                                                                                                                                                                  | Walk test—maximum voltage generated (KV) |                  |                  |
|-------------------------------------------------------------------------------------------------------------------------------------------------------------------------|------------------------------------------|------------------|------------------|
|                                                                                                                                                                         | Initial                                  | After 20M treads | After 40M treads |
| Control carpet (regular yarn-regular latex).....                                                                                                                        | 14.4                                     | —                | —                |
| Carpet with internal antistat yarn as defined in this invention.....                                                                                                    | 5.8                                      | 5.7              | 5.6              |
| Carpet with internal antistat yarn as defined in this invention in combination with latex containing five weight percent polyethylene oxide antistatic material.....    | 2.3                                      | 2.3              | 2.3              |
| Carpet with internal antistat yarn as defined in this invention in combination with latex containing five weight percent of the internal antistat used in the yarn..... | 2.2                                      | 2.2              | 2.2              |

#### Example 2

As in Example 1, except that the 6% antistatic agent containing an antioxidant is added by injection at the point where the molten polymer is extruded from the reactor prior to pelletizing. The subsequent washing cycles to extract any unreacted lactam and oligomers from the pellets did not effect the concentration of the antistat in the polymer as the antistat is insoluble in water. After washing and drying, the polymer was processed as in Example 1. The maximum voltage generated in KV in the Walk Test is 2.4 initially. It shows 2.2 after 20M treads and 2.0 after 40M treads.

#### Example 3

As in Example 1, except that 400 ends of undrawn yarn are combined into a tow. The tow is drawn, crimped and cut into 6.5 inch long staple, all in a continuous operation. The staple is then spun into a 2.25 with 3.5 "Z" twist and converted into 40 ounces/yd.² cut pile plush type carpets. The maximum voltage generated in KV in the Walk Test is 2.3. After 20M treads it dropped to 2.2 and after 40M treads it dropped to 2.01.

#### Example 4

As in Example 1, except that nylon 6,6 polymer is used. Continuous and staple yarns are prepared and the results in the carpets were as follows: initial KV is 2.9; after 20M treads, 2.1 KV; and after 40M treads the KV is 1.5.

#### Example 5

As in Example 1, except the yarn internal antistatic additive is added in an amount of 10 weight percent of the polymer. The resulting maximum voltage in the carpet is equivalent to results in Table I.

#### Example 6

As in Example 1, except the yarn internal antistatic additive is also used in the conductive latex. The resulting maximum voltage in the carpet is equivalent to results in Table I.

It is to be understood that although the instant invention has been described as set forth herein in a preferred form, obviously numerous modifications can be made without parting from the scope and spirit thereof, and such modifications are to be understood as coming within the scope of the appended claims.

We claim:

1. In a textile article comprised of an antistatic polyamide fiber a backing having said fiber secured thereto, and a coating on said backing contacting said fiber, said coating containing an additive to reduce buildup of static electricity

the improvement consisting essentially of using for said additive to reduce buildup of static electricity in said polyamide fiber between about 1 percent and about 12 percent by weight of a predominantly branched chain-extended compound represented by the formula



where  $a$ ,  $b$ ,  $c$ ,  $d$ ,  $w$ ,  $x$ ,  $y$ , and  $z$  are each a whole number and  $R$  is a difunctional radical from a hydrocarbon containing 1 to 13 carbon atoms, and at least one compound selected from the group consisting of diepoxides and compounds which yield the following divalent radicals:



where  $R'$  is a difunctional radical derived from aromatic, heterocyclic, cycloaliphatic or aliphatic hydrocarbons or combinations of them whereby said textile article will generate less than 3 kilovolts of static electricity by the walk test and the static electricity buildup gets lower with normal use of said textile article.

2. The article of claim 1 wherein the primary backing is made of synthetic material or jute.

3. The article of claim 1 wherein a secondary backing is added to said conductive latex backing, said secondary

backing is made up of spun-bonded or woven polypropyl material or jute.

4. The article of claim 1 wherein the polyamide is selected from the group consisting of polycaproamide and polyhexamethylene adipamide.

5. The article of claim 1 wherein the latex backing is styrene butadiene rubber latex.

10 6. The article of claim 5 wherein the latex contains up to ten weight percent of said latex of a compound selected from the group consisting of the reaction product of a compound as defined in claim 1 and polyethylene oxide.

7. The article of claim 6 wherein the antistatic efficacy improves with normal use.

15 8. The article of claim 1 wherein said additive to said coating is the same additive as is in said polyamide fiber.

#### References Cited

##### UNITED STATES PATENTS

- |    |           |        |                 |       |        |
|----|-----------|--------|-----------------|-------|--------|
| 20 | 3,554,824 | 1/1971 | Callahan        | ----- | 156-72 |
|    | 3,658,744 | 4/1972 | Brindell et al. | ----- | 161-62 |
|    | 3,510,386 | 5/1970 | Goins et al.    | ----- | 161-67 |
|    | 3,719,547 | 3/1973 | Martin et al.   | ----- | 161-67 |

25 HAROLD ANSHER, Primary Examiner

J. J. BELL, Assistant Examiner

U.S. Cl. X.R.

30 161-62